

# United States Patent

Forbes et al.

[15] 3,658,702

[45] Apr. 25, 1972

## [54] ORGANIC LOAD CARRYING ADDITIVE

[72] Inventors: **Eric Simon Forbes, Knaphill; Alan David Forbes, Woking, both of England**

[73] Assignee: **The British Petroleum Company Limited, London, England**

[22] Filed: **Nov. 26, 1969**

[21] Appl. No.: **880,308**

## [30] Foreign Application Priority Data

Dec. 6, 1968 Great Britain.....58,084/68

[52] U.S. Cl.....**252/49.9, 252/9, 252/32.5,**  
252/389, 252/400

[51] Int. Cl.....**C10m 1/46, C10m 1/32, C10m 3/40**

[58] Field of Search.....252/9, 32.5, 49.9, 389, 400

[56]

## References Cited

### UNITED STATES PATENTS

|           |        |                     |          |
|-----------|--------|---------------------|----------|
| 2,244,416 | 6/1941 | Ashburn et al. .... | 252/49.9 |
| 2,257,601 | 9/1941 | Hall et al. ....    | 252/49.9 |
| 2,285,854 | 6/1942 | Downing et al. .... | 252/49.9 |
| 2,400,120 | 5/1946 | Julian et al. ....  | 252/49.9 |
| 3,344,130 | 9/1967 | Mortenson. ....     | 252/400  |

### FOREIGN PATENTS OR APPLICATIONS

|           |         |                     |       |
|-----------|---------|---------------------|-------|
| 1,095,182 | 12/1967 | Great Britain ..... | 252/9 |
|-----------|---------|---------------------|-------|

*Primary Examiner—Daniel E. Wyman*

*Assistant Examiner—I. Vaughn*

*Attorney—Morgan, Finnegan, Durham & Pine*

[57]

## ABSTRACT

The lipid extract prepared by solvent extraction of micro-organisms when added to lubricating oils improve the load carrying, anti-oxidant, and anti-corrosion properties of the oils.

**4 Claims, 1 Drawing Figure**

PATENTED APR 25 1972

3,658,702



INVENTORS  
ERIC SIMON FORBES  
ALAN DAVID FORBES

BY

Morgan, Finnegan, Durkan & Pine  
ATTORNEYS

## ORGANIC LOAD CARRYING ADDITIVE

This invention relates to additives which can be added to lubricating oils to improve their properties, and to liquid lubricating compositions containing these additives. The additives of the present invention are produced from hydrocarbons by biochemical means.

It is known that it is possible to grow micro-organisms by the cultivation of micro-organisms on a hydrocarbon substrate in the presence of nutrient media and oxygen. The recovered micro-organisms may be purified by solvent extraction, and the purified micro-organisms are then available as food-stuff.

The waste products from the purification stage are a complex mixture of chemicals. Preferably the micro-organisms are yeasts.

We have now found that some of the waste products from the purification stage, referred to hereinafter as lipid extracts, when added to a lubricating base oil possess lubricating load-carrying properties, antioxidant and anti-corrosion properties.

According to the invention there is provided a composition which comprises a blend of a lubricating base oil and a lipid extract as hereinafter defined.

By lipid extract is meant that portion of a micro-organism culture grown on a hydrocarbon substrate which is separated from the micro-organism by solvent extraction.

In order to separate the lipid extract from the micro-organisms, a solvent system consisting of a polar and non-polar solvent may be used. Preferably the polar solvent contains a hydroxyl group. Suitable solvent systems are ethanol/diethyl-ether, methanol/chloroform, and isopropanol/n-hexane. Especially useful solvent systems are azeotropic mixtures of alcohols and hydrocarbons. Solvent systems consisting of alcohol/water mixtures are also useful, and the preferred solvent system is an azeotropic isopropanol/water system. The extraction may be carried out at room temperature.

Diethyl-ether may be used as a sole extractant but careful temperature control is required for efficient separation.

After the initial extraction of the lipid extract the solvents used can be evaporated off. When water is present in the solvent system an aqueous mixture is left which is then distilled to remove the water.

The hydrocarbons in which the yeast culture is grown are preferably petroleum fractions which can be obtained from crude oil. Preferably C<sub>10</sub> or higher straight chain hydrocarbons are present in, or constitute, the hydrocarbon in which the micro-organisms are grown, and preferably the hydrocarbon contains from 10-15 percent of straight chain paraffins. Suitable methods for growing yeast cultures are described in U.K. Pats. Nos. 914,567, 914,568, 101,7584, 1,011,7585, 1,021,697, 1,021,698, 1,049,065, 1,049,066, 1,049,067, 1,059,881, 1,059,886, 1,059,887, 1,059,891, 1,089,093, 1,095,182, 1,095,183.

The yeasts in this specification are classified according to the classification system outline in "The Yeasts, a Taxonomic Study" by J. Lodder and W.J.W. Kreger-Van Rij, published by North Holland Publishing Co. (Amsterdam) (1952).

Preferably when a yeast is employed this is of the family Cryptococcaceae and particularly of the sub-family Cryptococcoideae however, if desired there may be used, for example, ascosporeogenous yeasts of the sub-family Saccharomycoideae. Preferred genera of the Cryptococcoideae sub-family are Torulopsis (also known as Torula) and Candida. Preferred species of yeast are as follows. In particular it is preferred to use the specific stock of indicated Baarn reference number; these reference numbers refer to CBS stock held by the Central Bureau voor Schimmelculture, Baarn, Holland and to INRA stock held by the Institut National de la Recherche Agronomique, Paris, France.

|                   |                 |          |
|-------------------|-----------------|----------|
| <i>Candida</i>    | lipolytica      | CBS 610  |
| <i>Candida</i>    | pulcherrima     |          |
| <i>Candida</i>    | utilis          |          |
| <i>Candida</i>    | utilis, Variati |          |
| <i>Candida</i>    | major           |          |
| <i>Candida</i>    | tropicalis      | CBS 841  |
| <i>Torulopsis</i> | colliculosa     | CBS 2317 |
|                   |                 | CBS 133  |

|                   |             |              |
|-------------------|-------------|--------------|
| <i>Hansenula</i>  | anomala     | CBS 110      |
| <i>Oidium</i>     | lactis      |              |
| <i>Neurospora</i> | sitophila   |              |
| <i>Mycoderma</i>  | cancoillote | INRA: STV 11 |

- 5 Of the above *Candida lipolytica* is particularly preferred. If desired the micro-organism may be a mould. Suitable moulds are *Penicillium* and preferably there is used *Penicillium expansum*. Another suitable genus is *Aspergillus*.
- 10 If desired the micro-organism may be a bacterium. Suitably the bacteria are of one of the orders: *Pseudomonadales*, *Eubacteriales* and *Actinomycetales*. Preferably the bacteria which are employed are of the families *Corynebacteriaceae*, *Micrococcaceae*, *Achromobacteraceae*, *Actincymycetaceae*, *Rhizobiaceae*, *Bacillaceae* and *Pseudomonadaceae*. Preferred species are *Bacillus megaterium*, *Bacillus subtilis* and *Pseudomonas aeruginosa*. Other species which may be employed include: *Bacillus amylobacter*, *Pseudomonas natriegens*, *Arthrobacter* sp., *Micrococcus* sp., *Corynebacterium* sp., *Pseudomonas syringae*.
- 15 20 25 30 35 40 45 50 55 60 65 70 75
- Xanthomonas begoniae*, *Flavobacterium devorans*, *Acetobacter* sp., *Actinomyces* sp., *Nocardia opaca*. It will usually be possible to separate the micro-organism, contaminated with some unmetabolized feedstock and aqueous nutrient medium, from the bulk of the unmetabolized feedstock fraction. Preferably the separation is achieved by means of a decantation: additionally of alternatively centrifuging may be used.
- The preferred hydrocarbons in which the micro-organism is grown are the hydrocarbon gas oil fractions obtained from crude petroleum, and normal paraffins, e.g., those obtained from gas oil fractions e.g., by means of a molecular sieve separation process. The lipid extract obtained by the solvent extraction process is preferably subjected to further treatment to separate and concentrate the compositions possessing better load-carrying or anti-corrosion properties from the others. Suitable separation techniques include solvent fractionating, dialysis and chromatography.
- The first separation stage is preferably to remove any residual amounts of the hydrocarbon substrate, residual yeast or other impurities by shaking the lipid extract with an organic solvent preferably paraffin or ketone e.g., n-heptane or acetone to produce a purified lipid extract.
- The purified lipid extract can then be split into various further fractions to concentrate and separate the more useful fractions, and to obtain fractions which will be soluble in the base oil which is to be used.
- When it is desired to use the lipid extract as a load-carrying additive preferably the fractions containing the phospholipids are separated.
- A preferred way of carrying out a preparation of useful fractions is to carry out a further solvent extraction using a second solvent for example, petroleum ethers to obtain further extracts. By choice of this second solvent it is possible to separate the fraction which would be soluble in the base oil to which it is proposed to add the lipid extract.
- In a preferred method the solution obtained using the second solvent is contacted again with the first solvent to reprecipitate the dissolved lipid extracts. It has been found that this reprecipitated fraction is the most suitable for use in mineral base oils.
- The crude lipid extracts can also be split into various fractions by dialysis across a semi-permeable membrane, preferably a rubber membrane. This method can be used as an alternative to or in conjunction with the solvent extraction method and serves to purify and separate the more useful fractions of the crude lipid extracts.

The lubricating base oil preferably has a viscosity of 5 to 12 centistrokes at 210° F.

The lipid extract is preferably present in the lubricating oil/lipid extract blend in an amount of 0.05 to 10 percent by wt. and more preferably 0.1 to 5 percent.

It is a feature of the present invention that it enables a lubricating composition to be formed from a lubricating base oil and an additive which possesses load-carrying anti-oxidant and anti-corrosion properties.

Metal surfaces, especially ferrous surfaces, are liable to corrosion, and various additives have been added to oils coming into contact with such surface to inhibit this corrosion.

Corrosion inhibiting additives are especially useful for adding to oils which come into contact with water and which can be contaminated by water. This problem occurs particularly in lubricating oils for steam turbine bearings and gears. In these cases the contaminant is likely to be sea-water which can readily cause severe corrosion of unprotected surfaces.

It is very surprising that the lipid extracts produced by the growth of micro-organisms on a hydrocarbon substrate should be useful as lubricating oil additives.

The invention will now be described with reference to the following example.

#### EXAMPLE 1

A yeast of the family *Candida Tropicalis* was grown in a gas oil of boiling range 300° to 400° C. in the presence of a nutrient medium containing nitrogen and phosphorus. During the growth period air was blown through the liquid mixture. As described in U.K. Pat. No. 914,568.

When the growth had reached the desired stage as measured by the cellular density of the yeast the mixture was centrifuged. A pasty phase containing yeast cells impregnated with hydrocarbons and aqueous medium was thus separated. This pasty phase was washed with water to remove the bulk of the gas oil, and the product obtained heated to 80°-90° C. in a rapid current of air and ground to a powder.

The powder was treated by solvent extraction using a mixture of isopropanol, n-hexane and water. The solids not removed by the extracting liquids are the purified food-yeasts and the extracting liquids contain the yeast lipids extract. The extracting liquids can then be treated in two ways. If they are allowed to settle, two phases are formed, an upper phase containing isopropyl alcohol, n-hexane, any residual gas oil and some of the yeast lipids extract and a lower phase consisting of, mainly, isopropyl alcohol, water and the remainder of the yeast lipids extract. The solvents can be evaporated off from both these phases to yield yeast lipids fractions A.10 and B.11 as shown in the diagram. Alternately the extracting liquids can be subjected to distillation and all the solvent removed, prior to settling, to give a total yeast lipids extract, TL.9.

#### EXAMPLE 2

Lipids extract TL.9 prepared as in Example 1 was treated to the series of operations shown in the accompanying diagram. A number of fractions were thus obtained for testing as anti-wear additives.

The dialysis was carried out across a rubber membrane for 24 or 48 hours using n-hexane as a solvent.

The various fractions isolated were added to a liquid paraffin and the composition formed was tested in the Shell fourball tester and wear-scar diameter measured after 60 minutes. The results shown in the following Table 1 clearly demonstrate the anti-wear properties of the yeast lipid fractions, the tri-cresyl phosphate, a conventional anti-wear additive, is included as a comparison.

#### EXAMPLE 3

The total yeast lipid extract TL.9 prepared as in Example 1 was subjected to the following separation stages to isolate various fractions having enhanced anti-corrosion properties.

Crude lipids extract TL.9 was dissolved in n-heptane to yield TL.9.31 freed from residual yeast and mineral salts. As described in the accompanying diagram.

The various fractions of the lipid extract obtained as above were dissolved in several base oils and were tested using test procedures IP 135 A and IP 135 B. These tests indicate the ability of the oil compositions to prevent rusting of ferrous materials by oil compositions contaminated with water.

Test procedure IP 35 A uses distilled water and IP 35 B uses sea-water and is a more severe test.

The results are shown in the following Table 2, and the results to the amount of rusting seen in the test piece.

Samples TL 96 D and TL 918 D are prepared by the same steps. TL 96 B, TL 937 A, TL 954 A, and TL 958 A are prepared by the same steps and TL 96 C and TL 918 C are prepared by the same steps. The different batch numbers for the same fraction refer to different batches produced by the same process.

#### EXAMPLE 4

Lipid extract TL 931 prepared as in the diagram was tested as anti-oxidant in inhibiting the oxidation of a phenylene oxide. Compositions with and without TL 9.31 were shaken in a flask immersed in a silicone oil bath at 200° C. with air passing through the flask at constant mass flow. The decrease in oxygen content of the air from the test flask was measured. The induction period, maximum rate of oxidation and the total oxygen uptake were determined. The results are shown below.

Sample A Squalane (0.8 g.) plus polyphenylene oxide (2.3 g.)

Sample B Squalane (0.8 g.) plus polyphenylene oxide (2.3 g.) plus TL 9.31 (0.0147 g.) i.e. 1.8 percent weight.

Temperature 200° C., air flow rate 65 ml./min. duration 2 hours.

| Sample | Induction Period (mins) | Maximum Rate of Oxidation (mol O <sub>2</sub> mol <sup>-1</sup> sec <sup>-1</sup> ) | Total Oxygen Uptake (mol O <sub>2</sub> /mol squalane) |
|--------|-------------------------|-------------------------------------------------------------------------------------|--------------------------------------------------------|
| A      | 0                       | 0.55                                                                                | 2.3                                                    |
| B      | 16                      | 0.47                                                                                | 1.8                                                    |

The results show the antioxidant properties of the lipid extract.

TABLE 1

| Additive fraction used, 2% weight concentration | Nitrogen content of additive, percent weight | Phosphorus content of additive, percent weight | Wear scar diam. in mm. | Solubility in liquid paraffin |
|-------------------------------------------------|----------------------------------------------|------------------------------------------------|------------------------|-------------------------------|
| TL9.....                                        | 0.71                                         | 1.10                                           | 0.40                   | F                             |
| TL9(1)3A.....                                   | 3.2                                          | 5.10                                           | 0.34                   | S                             |
| TL93B.....                                      | 0.21                                         | 0.1                                            | 0.66                   | S                             |
| TL93A.....                                      | 1.68                                         | 2.14                                           | 0.33                   | S                             |
| TL96B.....                                      | 2.05                                         | 4.7                                            | 0.41                   | F                             |
| TL96C.....                                      | 1.4                                          | 2.9                                            | 0.37                   | S                             |
| B113A.....                                      | 3.23                                         | 2.90                                           | 0.55                   | F                             |
| None.....                                       | Nil                                          | Nil                                            | 0.75                   |                               |
| Tri-cresyl phosphate.....                       | Nil                                          | 8.42                                           | 0.35                   | S                             |
| TL9(2).....                                     | 0.70                                         | 10.6                                           | 0.38                   | S                             |
| TL9(2).....                                     | 0.70                                         | 1.06                                           | 0.34                   | S                             |
| TL9(2)**.....                                   | 0.70                                         | 1.06                                           | 0.44                   | S                             |

F means that suspension of the additive in the liquid paraffin was filtered.

S means that the additive was soluble in liquid paraffin.

\*0.5 percent weight concentration.

\*\*0.05 percent weight concentration.

TABLE 2

| Additive | Amount by wt. | Base Oil        | Amount of Corrosion using test methods |          |
|----------|---------------|-----------------|----------------------------------------|----------|
|          |               |                 | IP 135 A                               | IP 135 B |
| None     | —             | liquid paraffin | 100%                                   | 100%     |
| TL 96 B  | 0.3%          | liquid paraffin | Nil                                    | —        |
| TL 918 D | 0.5%          | liquid paraffin | Nil                                    | —        |

|          |      |                 |     |       |
|----------|------|-----------------|-----|-------|
| TL 918 A | 0.5% | liquid paraffin | —   | 15%   |
| TL 918 A | 1.0% | liquid paraffin | —   | Nil   |
| TL 918 A | 2.0% | liquid paraffin | —   | Nil   |
| TL 954 A | 1.0% | liquid paraffin | —   | 4%    |
| TL 958 A | 1.0% | liquid paraffin | —   | Nil   |
| TL 931   | 2.0% | liquid paraffin | —   | Nil   |
| TL 954 A | 2.0% | HB 125          | —   | 15%   |
| TL 937 A | 1.0% | BG 160/95       | Nil | 4%    |
| TL 937 A | 2.0% | BG 160/95       | —   | Spots |
| TL 958 A | 1.0% | BG 65/100       | —   | Nil   |

In the table the base oil HB 125 was a solvent refined base oil of viscosity of 125 Redwood No. 1 secs. at 140° F. the base oil BG 160/95 was lubricating base oil of viscosity 160 Redwood No. 1 secs. at 140° F. and a viscosity index of 95 and the base oil BG 65/100 was a lubricating base oil of viscosity 6 Redwood No. 1 secs. at 140° F. and a viscosity index of 100.

The lipid extracts used showed marked ability to reduce corrosion even in the sever IP 135 B test.

We claim:

1. A lubricating composition which comprises a lubricating base oil and from 0.05 through 10 percent by weight based on the total weight of the composition of a lipid extract containing nitrogen and phosphorus and obtained by the solvent extraction of a micro-organism culture grown on a hydrocarbon substrate.

2. A lubricating composition as claimed in claim 1 in which the said liquid extract is contacted with an organic liquid selected from paraffins and ketones to precipitate a purified lipid extract which is incorporated in the said base oil.

3. A lubricating composition as claimed in claim 1 in which the lubricating base oil has a viscosity of 5 to 12 centistrokes at 210° F.

4. A lubricating composition as claimed in claim 1 in which the said hydrocarbon substrate is selected from gas oil fractions obtained by the distillation of crude petroleum and normal paraffins, and in which the micro-organism is a yeast.

\* \* \* \* \*

20

25

30

35

40

45

50

55

60

65

70

75

UNITED STATES PATENT OFFICE  
CERTIFICATE OF CORRECTION

Patent No. 3,658,702

Dated April 25, 1972

Inventor(s) Eric Simon Forbes and Alan David Forbes

It is certified that error appears in the above-identified patent and that said Letters Patent are hereby corrected as shown below:

- Column 1, line 49, "101,7584" should read -- 1,017,584 --;
- Column 3, line 2, "centistrokes" should read --centistokes--;
- Column 4, Table I, under the heading "Phosphorus content..." and on the line beginning with "TL9(2)", "10.6" should read -- 1.06 --; and
- Column 5, line 15, "viscosity 6" should read -- viscosity 65 --.

Signed and sealed this 25th day of July 1972.

(SEAL)

Attest:

EDWARD M. FLETCHER, JR.  
Attesting Officer

ROBERT GOTTSCHALK  
Commissioner of Patents